

Patented Sept. 26, 1922.

1,430,163

## UNITED STATES PATENT OFFICE.

HEINRICH FORSTER, OF BRUGGEN, SWITZERLAND, ASSIGNOR OF ONE-HALF TO  
CONRAD FORSTER, OF DEDHAM, MASSACHUSETTS.

### PROCESS FOR IMPARTING TRANSPARENT EFFECTS TO COTTON.

No Drawing.

Application filed September 21, 1920. Serial No. 411,849.

To all whom it may concern:

Be it known that I, HEINRICH FORSTER, a citizen of the Swiss Republic, residing at Bruggen, Canton St. Gallen, Switzerland, 5 have invented certain new and useful Improvements in Processes for Imparting Transparent Effects to Cotton; and I do hereby declare the following to be a full, clear, and exact description of the invention, 10 such as will enable others skilled in the art to which it appertains to make and use the same.

This invention relates to a process for imparting transparent effects to cotton.

15 The object of the invention is to provide a novel process by which superior transparent effects may be imparted to cotton, cotton fabrics, and mixed fabrics containing cotton.

It has heretofore been recognized that certain transparent effects may be imparted to 20 cotton by successive treatments of the cotton with reagents of different types and characteristics, having different actions upon cotton, and of which strong sulphuric acid and 25 concentrated soda lye may be taken as examples of each type. To produce such effects

the cotton was either treated first with 30 strong sulphuric acid for a few seconds followed by treatment with strong soda lye or,

35 on the other hand, the cotton was treated first with strong soda lye and then with strong sulphuric acid for a few seconds. The concentration of the sulphuric acid was over 50 $\frac{1}{2}$ ° Baumé. It has also been recognized

40 that the transparent effects secured by these processes could be improved to some extent by preceding the initial step in each process with a treatment of the cotton with a reagent of the opposite type from the reagent

45 used in the initial step of the process, that is to say, the first process consisting of a treatment with sulphuric acid followed by a treatment with soda lye was improved by preceding the treatment with sulphuric acid

50 by a treatment with strong soda lye, and also the process consisting of the treatment with soda lye followed by treatment with strong sulphuric acid, was improved by preceding the soda lye treatment with treatment

esses may be symbolically expressed as follows:



In both processes the initial treatment with strong sulphuric acid or strong soda lye appears to operate to prepare the material and place it in a condition more favorable to the successful operation of the subsequent treatments. It is to be noted that the first two treatments in each of processes 55 1 and 2 are with reagents of opposed types.

It has heretofore been considered impossible to obtain any reaction or effect upon cotton by successive treatments with reagents of the same general type, that is for example by successive treatments with reagents having an action upon cotton similar to sulphuric acid.

60 I have discovered that transparent effects of superior and improved quality may be produced upon cotton by successive treatments with reagents of the same general type but under different conditions of operation.

70 The conditions of operation under which the cotton is treated with reagents of one type may be varied in several ways, for example, successive treatments of cotton with acids of different strengths followed by treatment with strong soda lye produced transparent effects upon cotton vastly superior to those produced by any of the processes heretofore known. Different reagents 75 of the same type may be used in each of the successive steps but under different conditions of operation. Instead of varying the strength of the reagent to be used in a particular treatment, the temperature thereof 80 may be controlled with or without variation in its strength. It has been heretofore recognized that in general the effectiveness of a reagent is in a large measure dependent upon its temperature. It is therefore possible 85 to obtain desirable transparent effects by treatment with a reagent of one type at one temperature, treatment with the same reagent or a reagent of the same type at another temperature followed by treatment 90

95 100

with a reagent of a different type. The conditions of operation may be varied in other ways.

The invention is preferably embodied in the following process which is described in detail as follows:

The cotton fabric is dipped in sulphuric acid of a strength corresponding to pure sulphuric acid having a gravity below  $50\frac{1}{2}^{\circ}$  Baumé. The exact strength of this acid may be varied within reasonable limits and is preferably a strength corresponding to sulphuric acid of a gravity of  $49\frac{1}{2}^{\circ}$  Baumé.

The cotton is permitted to remain in this acid bath for a period of approximately two minutes after which it is removed therefrom, washed thoroughly, and dried. The cotton is then dipped into a second sulphuric acid bath for a period of a few seconds, preferably four or five, and the strength of this second bath corresponds to pure sulphuric acid having a gravity above  $50\frac{1}{2}^{\circ}$  Baumé, and preferably  $54^{\circ}$  Baumé. After the cotton has remained in this second acid bath for a period of approximately five seconds, it is removed therefrom and washed, and thereafter mercerized in the usual way in a bath of soda lye of a strength above  $15^{\circ}$  Baumé. This process may be symbolically expressed as follows:

$H_2SO_4$  below  $50\frac{1}{2}^{\circ}$  Bé.— $H_2SO_4$  above  $50\frac{1}{2}^{\circ}$  Bé.—NaOH.

During the process shrinkage of the material is prevented as much as possible so that the material is in a stretched condition.

The superiority of the transparent effects produced upon the cotton material treated in accordance with the present invention may be readily observed by comparison with fabrics treated according to previous processes. The fabrics treated according to the present invention are far more transparent, more even, and more silk-like.

Among the reagents having an action upon cotton similar to sulphuric acid, and which may be employed in accordance with the present invention are included phosphoric acid, hydrochloric acid, nitric acid or any mixtures thereof including mixtures with sulphuric acid, and also zinc chloride solution and ammoniacal solutions of copper hydrate. All of these reagents may be regarded as parchmentizing reagents.

The cotton material may be treated in any desired manner in accordance with the present process either in whole or in part in order to produce the pattern effects according to the well-known printing process.

In the specification and claims the gravity

of solutions expressed in degrees Baumé are 00 to be considered as degrees Baumé at a temperature of approximately  $15^{\circ}$  C.

Having thus described the invention, what is claimed is—

1. The process of imparting transparent effects to cotton which consists in subjecting the cotton to treatment with successive parchmentizing reagents under different conditions of operation and thereafter mercerizing the cotton. 05

2. The process of imparting transparent effects to cotton which consists in subjecting the cotton, while in a stretched condition, to treatment with successive parchmentizing reagents under different conditions of operation and thereafter mercerizing the cotton. 75

3. The process of imparting transparent effects to cotton which consists in subjecting particular portions of the cotton to treatment with successive parchmentizing reagents under different conditions of operation and thereafter mercerizing the cotton. 80

4. The process of imparting transparent effects to cotton which consists in subjecting the cotton to treatment with successive parchmentizing reagents of different strengths, and thereafter mercerizing the cotton. 85

5. The process of imparting transparent effects to cotton which consists in subjecting the cotton to treatment with successive parchmentizing reagents of different and increasing strengths, and thereafter mercerizing the cotton. 90

6. The process of imparting transparent effects to cotton which consists in subjecting the cotton to treatment first with sulphuric acid below  $50\frac{1}{2}^{\circ}$  Baumé, then with sulphuric acid above  $50\frac{1}{2}^{\circ}$  Baumé and then with concentrated caustic alkali. 95

7. The process of imparting transparent effects to cotton which consists in subjecting the cotton to treatment for a period of substantially two minutes with sulphuric acid having a gravity between  $45-50\frac{1}{2}^{\circ}$  Baumé, 105 washing and drying the cotton, then subjecting the cotton to treatment for a few seconds with sulphuric acid having a gravity above  $50\frac{1}{2}^{\circ}$  Baumé, washing and thereafter mercerizing the cotton in concentrated 110 soda lye.

8. The process of imparting transparent effects to cotton which consists in subjecting the cotton to successive parchmentizing and mercerizing treatments, one of such treatments being carried out in two successive steps under different conditions of operation. 115

HEINRICH FORSTER.